

G. H. ELLIS.  
INSULATING FABRIC.  
APPLICATION FILED MAR. 19, 1910.

1,108,155.

Patented Aug. 25, 1914.



WITNESSES

E. C. Skinkle

B. M. Wheeler

INVENTOR  
George H. Ellis  
BY HIS ATTORNEYS

Williamson, Michaud

# UNITED STATES PATENT OFFICE.

GEORGE H. ELLIS, OF ST. PAUL, MINNESOTA, ASSIGNOR, BY MESNE ASSIGNMENTS, TO NORTHERN INSULATING COMPANY, OF ST. PAUL, MINNESOTA, A CORPORATION OF MINNESOTA.

## INSULATING FABRIC.

1,108,155.

Specification of Letters Patent.

Patented Aug. 25, 1914.

Application filed March 19, 1910. Serial No. 550,359.

To all whom it may concern:

Be it known that I, GEORGE H. ELLIS, a citizen of the United States, residing at St. Paul, in the county of Ramsey and State of Minnesota, have invented certain new and useful Improvements in Insulating Fabric; and I do hereby declare the following to be a full, clear, and exact description of the invention, such as will enable others skilled in the art to which it appertains to make and use the same.

My invention has for its object to provide, as a new article of manufacture or product, a felted or matted fibrous insulating fabric.

15 The present improved product is in the nature of an improvement on the product disclosed and broadly claimed in Patent No. 908,681, issued of date January 5, 1909, to James E. Lappen, and entitled "Flax felt."

20 In the said prior Lappen patent, the so-called flax felt is made from long fibers that are intertwined and matted together, so that they constitute a porous, coherent and self-sustaining body having considerable tensile

25 strength. This is also true of the present improved product. Also, in common with the material defined in the said patent, the flax or other fiber, from which the body of the fabric is made, is degummed or partly

30 degummed, so as to separate the shive from the fiber; and a part, usually about fifty per cent., more or less, of the shive or woody substance, is commingled with the fiber. This

35 use of the shive renders the felted material more porous than it would be if entirely freed from shive and, furthermore, greatly reduces the cost of the manufactured material.

40 The present improved product differs from the product of the said patent chiefly in the following important features: The cordices or fibrous bundles of the flax or similar fibrous material are not only partially separated as in the product of the said prior

45 patent, but are shredded or frayed so that they are formed with beard or fuzz which very closely unite and very thoroughly intertwine and form, in the insulating material, a very strong mechanical binder made up of

50 fluffy and very soft and light body portions which also serve to very greatly increase the heat insulating capacity of the completed fabric or felted material.

55 The invention is illustrated in the accompanying drawing which represents more or

less diagrammatically a cross section of a portion of the improved product.

In the drawing, the cordices or fibrous bundles hereinbefore referred to are indicated by the heavy black lines and are designated by the numeral 1. The beard or fuzz formed upon the fibers 1 is indicated at 2, the strands of which intertwine with each other and with adjacent fibers, as shown in the drawing.

Actual practice has demonstrated that my improved insulating fabric or felted board of a given thickness will have higher heat insulating efficiency, will be lighter in weight and yet much tougher and coherent

60 or self-sustaining in its nature than a felted board or material of the same thickness made as described in the said prior Lappen Patent 908,681.

65 The shredded or frayed beard or fuzz of the fiber so thoroughly intertwine that they bind together not only

themselves but the coarser fibers and the shive and, hence, their high efficiency as a

50 mechanical binder. The lightness of the material is due to the fluffy nature of a large

55 part of the material which is made up of the intertwined fuzz or beard; and the increased insulating efficiency seems to be due

60 largely to the greatly increased number of very small air cells produced in the material

65 by the said intertwined fuzz or beard. To

70 produce this shredding or fraying of the fibrous stock with the resulting beard or fuzz

75 thereon, and to remove the pectose or gum, at least in part, from the stock, the fibrous

80 stock is subjected to a carding action under water, this action being a feature which is

85 disclosed and broadly claimed in my companion application, Serial No. 550,360 filed

90 of even date herewith and entitled "Process

95 of producing insulating fabric." In fact,

100 my said process application discloses a complete process, by means of which this improved insulating fabric may be commercially made. In my prior Patent, No.

105 1,022,778 of April 9, 1912, I have disclosed

110 an apparatus which is adapted for use to commercially and economically carry out the improved process of making my improved insulating fabric.

What I claim is:

1. An insulating fabric composed of shredded and fibrous stock felted together the fibers being provided with a beard or fuzz, said beard or fuzz being intertwined

110

and matted to provide a reinforcement in addition to that resulting from the felting of the fibers.

2. An insulating fabric composed of long partly degummed fiber and shive or woody particles, the said fibrous portions being shredded or frayed and formed with a beard or fuzz intertwined and matted together to provide a reinforcement in addition to the reinforcement resulting from the felting.

3. An insulating fabric composed of shredded and fibrous stock felted together the fibers being provided with a beard or

fuzz, the beard or fuzz on each fiber being intertwined both with the beard or fuzz on 15 adjacent fibers and with the adjacent fibers themselves, thereby providing a reinforcement in addition to that resulting from the felting of the fibers.

In testimony whereof I affix my signature 20 in presence of two witnesses.

GEORGE H. ELLIS.

Witnesses:

ALICE V. SWANSON,  
HARRY D. KILGORE.